

June 6, 1939.

W. C. VAN GEEL

2,161,600

ELECTRODE SYSTEM FOR RECTIFYING OR CONTROLLING HIGH  
OR INTERMEDIATE FREQUENCY OSCILLATIONS

Filed June 20, 1936

*Fig. 1*



*Fig. 2*



*Fig. 3*



INVENTOR  
W. C. VAN GEEL

BY *H. S. Grover*  
ATTORNEY

## UNITED STATES PATENT OFFICE

2,161,600

ELECTRODE SYSTEM FOR RECTIFYING OR  
CONTROLLING HIGH OR INTERMEDIATE  
FREQUENCY OSCILLATIONS

Willem Christiaan van Geel, Eindhoven, Netherlands, assignor to N. V. Philips' Gloeilampenfabrieken, Eindhoven, Netherlands, a corporation of the Netherlands

Application June 20, 1936, Serial No. 86,288.  
In Germany July 30, 1935

6 Claims. (Cl. 175—366)

This invention relates to an electrode system for rectifying or controlling high or intermediate frequency oscillations, in which a preferably separate insulating coating is provided between the electrodes.

With this kind of electrode system an electro-negative electrode consisting of semi-conductive material is provided. This material is bounded on at least one side by an insulating coating (in 10 which one or more grids may be provided) having a very small thickness (of the order of magnitude of 0.1 to  $10\mu$ ) on to which a well conducting electrode is applied. It may be advantageous to provide this insulating coating separately.

Such an electrode system has various advantages when used, for instance, in radio receiving or television apparatus. A rectifying effect of the system when used as a detector can be readily obtained by means of a comparatively low voltage applied to the electrodes, this voltage on account of the said very small thickness of the insulating coating being capable of setting up an electric field of considerable intensity between the electrodes.

However, such an electrode system for rectifying or controlling high or intermediate frequency oscillations has the drawback that it is possessed of a comparatively high self-capacity.

This capacity depends either on the size of the contact surface between the well conducting electrode and the insulating coating, or on the size of the contact surface between the semi-conductive electrode and the insulating coating, or again on the size of the contact surface between the semi-conductive electrode and the supply conductor, for in the latter case substantially only that column of the semi-conductive electrode, whose section substantially corresponds to the said contact surface between this electrode and the supply conductor, partakes in the conduction.

According to the invention the drawback of a high self-capacity is avoided by forming at least one of the system parts determining the capacity of the system in such a manner by means of a mass in the liquid state, that the contact surface determining the capacity is reduced to a surface not exceeding  $10 \text{ mm}^2$ , either by the surface tension of the mass applied in an exact small quantity, or by an envelope arranged about said mass on the contact surface. The liquid mass may either consist of the molten electrode material, or may contain it, for instance, as a chemical compound in the dissolved or suspended state.

It has already been proposed to incorporate a

crystal acting as a detector in a radio receiving set. A crystal detector exhibits a rectifying effect only at one or some points of the crystal surface and more particularly where an insulating coating is available on the surface which 5 coating must have such a thickness that its resistance does not have an excessive value and corresponds to the applied voltage to be rectified. Thus, when using a crystal as a detector the crystal surface must be scanned with the aid of 10 a pointed metal contact until a point possessing a rectifying effect has been found.

This drawback is not inherent to electrode systems according to the present invention. In these systems any point of the insulating coating 15 has a rectifying effect, if on either side of the insulating coating there is a point of one terminal electrode that lies opposite a point of the other terminal electrode.

Since the thickness of the insulating coating 20 in an electrode system according to the invention is determined beforehand and the whole contact surface has a detector effect, the capacity may be arbitrarily chosen.

The same holds good when the electrode system 25 is used for controlling oscillations.

It has already been proposed to provide a truncated lead cone on a cuprous-oxide detector, which cone serves as a supply conductor for one of the electrodes. In this case the capacity 30 depends on the surface of the graphite layer available under the lead cone. In this manner it is very difficult to obtain a small surface capable of being reproduced with such a graphite layer.

The present invention permits the self-capacity 35 of an electrode system or cell to be made extremely low. However, in contra-distinction to the prior art, by reason of the means used according to the invention for obtaining the desired effect, it is possible to determine beforehand the definite value of the self-capacity of the cell which is capable of being reproduced. In view of the fact that the self-capacity has a definite influence on a circuit comprising the cell it is of great importance that the self-capacity 40 of such cells has the same value and is capable of being reproduced. In order to ensure the most favorable operation in such a circuit certain measures are taken when designing it. If the self-capacity of the cells would be different, then 45 in spite of the fact that certain measures have been taken, these measures could not bring out themselves if the initial cell adapted to the circuit would be replaced by another one.

The electrode system according to the inven- 55

tion has the further advantage that it requires only an extremely small space due to its compact construction, which may be of advantage in a radio set, and by surrounding it with compound 5 mass it may constitute a firm assembly.

In contradistinction to the usual radio valves these electrode systems do not require any cathode heating power.

The conductors supplying this energy, for instance, to the detector tube, determine the location of this tube in a modern receiver. However due to the disturbing effect exerted, for instance, on the high frequency part, the source of alternating current heating power cannot be provided at optional points in such receivers. 15

These supply conductors being obviated, the problem of the arrangement of a detector according to the invention is greatly simplified, since it may be provided where it is most suitable in view of the smallest length of the connecting wires. Owing to its small size and weight such a system may be suspended and mounted in the wiring itself. 20

The invention will be more clearly understood 25 by reference to the accompanying drawing wherein Figs. 1, 2 and 3 illustrate enlarged views of various modifications of the electrode systems according to the present invention.

For the semi-conductive (electro-negative) 30 electrode 1 (Figure 1) cuprous sulphide-(Cu<sub>2</sub>S) is used, which is applied as such on a brass support 2 by pressing. After that the semiconductor is coated with an insulating polystyrene coating 3 which may be effected by immersing it in 35 a bath containing insulating coating material dissolved in benzene and by slowly drawing it out of this bath. In accordance with the voltage to be blocked a thickness of 1 to 10 $\mu$  may be used.

On the insulating coating is placed a tube 4 of 40 quartz whose bore extends conically towards the bottom side so that the aperture 5 is about 0.125 mm.<sup>2</sup>.

This tube perfectly adheres to the insulating coating 3 when the material of the insulating 45 coating itself is used as an adhesive. In this case heating up to more than 100° C., for instance, may be necessary. The supply conductor 6 is inserted into this tube and after that the tube 4 is filled with a metal suspension 7 such as a suspension 50 of platinum in alcohol, or with a colloidal graphite solution (for instance, the colloidal graphite solution in water sold under the registered trade-mark "Aquadag"). After concentration by evaporation of the suspension 55 agent the good conductive electrode 1 which is constituted by the solid residue is connected both mechanically and electrically to the supply conductor 6. Instead of a metal suspension it is also possible to use a solution of a chemical compound of a metal, the chemical compound being reduced. It is possible, for instance, to use 60 one of the well known silver solutions such as an ammoniacal silver solution to which glucose is added.

If desired, the tube 4 may be removed after the 65 good conductive electrode has been formed.

The following method of manufacture concerns a detector (Figure 2) wherein the negative electrode consists of selenium.

A definite quantity of the liquid selenium 9 is 70 applied on to a brass plate 8 and after cooling down it is covered with an insulating coating 10 of artificial resin which covers also the brass side where the selenium is provided as appears from 75 the drawing.

The support together with the selenium and the insulating coating provided thereon is introduced into a furnace and heated for some time (generally 2 to 24 hours) at a temperature of about 200° C. This operation has for its purpose 5 to convert the selenium into the conductive crystalline modification. When the synthetic resin used for the coating layer is polystyrene then heating has the additional advantage that the polystyrene can be polymerised thoroughly, 10 thus improving the favorable dielectric properties.

On to the insulating coating a definite quantity of Rose metal 11 (50 Bi, 27.1 Pb, 22.9 Sn) is applied which is arranged at the level of the 15 spherical selenium part 9. The metal 11 will contact with the insulating coating over a limited surface only (for instance 0.25 mm.<sup>2</sup>). This surface can be previously determined and depends on the surface tension and the quantity of 20 material.

While the drop 11 is still in liquid form a supply conductor 12 is immersed which after solidification of the electrode material ensures a perfect mechanical and electrical joint. 25

Both the above examples relate to the manufacture of electrode systems wherein the semi-conductive electrode is applied in the form of a thin layer on to a flat plate, whereas the good conductive electrode is formed inside an envelope or as a definite drop. Hereinafter the manufacture of a system according to the invention will be set out by reference to Figure 3, in which the selenium, i. e., the semi-conductive electrode is provided in a pearl-shaped envelope. 30

Graphite 14 is provided in a steatite pearl 13 having a cylindrical bore of about 0.5 mm. up to a distance of about 0.03 mm. from the upper edge. This graphite assures a perfect contact with the selenium 15 to be applied thereon. At 40 16 the graphite is electrolytically coppered in order that a supply conductor can be soldered thereto.

After that the cavity of the pearl above the graphite is filled with liquid selenium 15. A 45 smooth surface and a uniform thickness of the layer can be obtained by striking, for instance, a razor over the selenium while it is in the liquid state.

Thereupon an insulating coating 17 is formed 50 on the selenium and, if desired, on the whole surface of the pearl, by immersion into a solution of polystyrene in benzene. After this treatment the assembly is heated at about 200° C. as has been set out in the last-mentioned example. 55

The counterelectrode 18 provided on the insulating coating 17 is constituted by a definite metal quantity having a low melting point such as Wood's metal (50 Bi, 25 Pb, 12.5 Sn, 12.5 Cd), in which the conductor 19 is inserted, while the 60 drop is in liquid form, so that the conductor is secured upon solidification.

In the above examples a pearl is used for enveloping the electrode material, this pearl surrounding either the semi-conductor or the good 65 conductive electrode.

It will be appreciated that each electrode, both the good emitting electrode and the semi-conductive electrode, may be mounted in a pearl. In this case the pearls may be agglutinated together with the aid of polystyrene, thus obtaining not only a very favorable insulation between both the electrodes, but also a good mechanical joint because polystyrene is an excellent adhesive. 70

In order to render the assembly more rigid and 75

to secure the supply conductors mechanically in a suitable manner such an electrode system, if required after having been inserted in a tube, is filled up with compound mass. In this manner the supply conductors bear in the compound mass so that the connecting points of the electrodes are not liable to mechanical stresses.

Also other methods of manufacturing electrode systems fall within the scope of the invention as defined by the appended claims.

What I claim is:

1. An electrode system for rectifying or controlling high or intermediate frequency electrical oscillations, comprising an electro-positive electrode of an alloy composed of at least bismuth, lead and tin and an electro-negative electrode of selenium, an insulating coating of polystyrene provided between the electrodes, and characterised in that at least one of the capacity determining parts of the system is formed with the aid of a mass in the liquid state in such a manner that the contact surface determining the electrostatic capacitance is limited to a surface not exceeding 10 mm.<sup>2</sup>.
2. An electrode system as claimed in claim 1, in which the portion yielding the surface determining the capacity is applied in the molten state.
3. An electrode system comprising a pair of

main electrodes, one of which is electro-positive and is made of an alloy composed of at least bismuth, lead and tin, and the other of which is electro-negative and is made of selenium, and a thin insulating layer of polystyrene interposed 5 between and contacting the surfaces of the main electrodes.

4. An electrode system according to claim 3 wherein the electro-positive electrode is made of Rose metal.

5. An electrode system according to claim 3 wherein the electro-positive electrode is made of Wood's metal.

6. An electrode system comprising a cylinder having a central bore, a filling of graphite within the bore except for a short distance from the upper surface of the cylinder, a quantity of selenium constituting the negative electrode of the system deposited within the remaining portion of the bore between the graphite filling and 15 the upper surface of the cylinder, a thin layer of polystyrene contacting with the upper surfaces of the cylinder and the selenium electrode, a quantity of Wood's metal constituting the positive electrode of the system contacting with the 20 polystyrene layer on the side opposite to the negative electrode, and a lead connected to each of the electrodes.

WILLEM CHRISTIAAN VAN GEELEN.